

# UNITED STATES PATENT OFFICE.

WALDEMAR BRUNO, OF BERLIN, GERMANY.

## MANUFACTURING INCANDESCENCE BODIES.

1,051,677.

Specification of Letters Patent.

Patented Jan. 28, 1913.

No Drawing.

Application filed July 6, 1909. Serial No. 506,030.

*To all whom it may concern:*

Be it known that I, WALDEMAR BRUNO, engineer, residing at N. Liebenwalderstrasse 10, Berlin, Germany, have invented certain 5 new and useful Improvements in the Manufacturing of Incandescence Bodies; and I do hereby declare the following to be a full, clear, and exact description of the invention, such as will enable others skilled in the art 10 to which it appertains to make and use the same.

The present invention relates to the manufacture of incandescent bodies for gas burners, from artificial filaments, to which the 15 requisite salts of the rare earths are applied in the form of solutions, as in the case of incandescent bodies of cotton or other vegetable fibers.

The impregnation of incandescence bodies 20 of artificial filaments does not itself present any difficulty, but considerable difficulties have been encountered in the burning of such bodies, owing to the absence of a strong skeleton of ash, and to the conversion of 25 nitrates into oxids, accompanied by swelling injurious to the structure. To obviate this it is essential to arrange that the formation of oxid is not due solely to the action of the flame, but is at least in part procured 30 in advance with the aid of suitable chemical reactions. By this means there is formed a skeleton consisting of the oxids or hydrates of the salts which very quickly bakes or fuses together in the flame and gives the 35 necessary strength to the structure.

This process consists in treating the impregnated mantles in a bath at a temperature of about 40 or 50° C. This bath consists of a mixture of alkalis or amins and 40 acid which are capable, with coöperation of the bases, to convert the nitrates into basic double compounds. Acetic acid, oxalic acid and other organic acids may be used; also phenols. The alkalis or amins used must 45 form volatilizable compounds and soluble compounds with the said acids and with the nitric acid of the salts of the rare earths. The formation of the basic double compounds is materially favored by immersing 50 the moist fabric into the heated solutions of alkali or amin at the moment at which the acid is added, and at which considerable heat of formation is evolved. The conversion of the nitrates into insoluble or nearly 55 insoluble compounds takes place almost in-

stantaneously, so that no lixiviation of salts can take place. If the alkalis or amins are present in excess the basic double salts are more or less converted into oxids or hydrates. The employment of an excess of 60 alkali is, however, not necessary since when the body is ignited the basic double salts are easily converted into oxids of the rare earth metals, without swelling, since the acids used are easily vaporizable. 65

A suitable bath for treating the impregnated fibrous fabric is prepared as follows: Two kilograms of crystallized oxalic acid are dissolved in twenty kilograms of distilled water at a temperature from 70 to 75° C. 70 and ten kilograms of liquid ammonia of normal temperature are added to this solution. At the moment, when the chemical action takes place in the so prepared bath (which consists of the compounds of the 75 chemical combination of oxalic acid with the alkali), the impregnated stockings are thrown in and properly immersed in the solution. At this point the solution must be kept at a temperature between 40 to 80 50° C. The mantles are kept in the solution at this temperature for about two minutes. (It may be noted that at 37° C. the salts are precipitated.)

The incandescence bodies produced are of 85 great tensile strength capable of bearing 50 to 60 grams and are elastic and flexible.

Since the final treatment takes place in *statu nascendi*, the chemical reactions are rapid. Consequently there is no loss of rare 90 earths, and the bodies are of extremely uniform composition, and are also characterized by great uniformity of lighting power. The rapidity of the reaction is increased by the treatment of the bodies in a somewhat moist 95 state, as described.

Having thus described my invention, I declare that what I claim as new and desire to be secured by Letters Patent is:

A process for making incandescence bodies 100 from artificial filaments, which consists in first impregnating the filaments with the requisite nitrates of the rare earths, then treating the impregnated filaments while moist with a mixture of such alkalis or 105 amins and acids as are capable, with the coöperation of the bases, of converting the nitrates into basic double salts, and which form volatilizable compounds and soluble compounds with the nitric acid of the salts 110

of the rare earths, said impregnated filaments being immersed in the mixture at the time the acid is added to it and heat is thereby evolved, and maintaining the solution and filaments at a temperature between 40° and 50° C. for a relatively short period of time.

In testimony whereof I affix my signature, in presence of two witnesses.

WALDEMAR BRUNO.

Witnesses:

WALDEMAR HAUPT,  
HENRY HASPER.

---

Copies of this patent may be obtained for five cents each, by addressing the "Commissioner of Patents, Washington, D. C."

---